

# United States Patent Office

3.296.101

Patented Jan. 3, 1967

1

3.296.101

3,296,101

# CYANIDE ELECTROPLATING BATHS AND PROCESSES

James R. Crain, Penn Hills, Pa., assignor, by mesne assignments, to Cowles Chemical Company, Shaker Heights, Ohio, a corporation of Ohio  
No Drawing. Filed Feb. 25, 1963, Ser. No. 260,823  
19 Claims. (Cl. 204—44)

This invention relates to the deposition of metals from cyanide metal plating baths and has particular reference to novel electrolytes and processes associated therewith which will produce brighter and smoother metal electrodeposits.

Numerous compounds, singly and in combination, are employed as additives in the cyanide electrolytes from which metals such as copper, brass, bronze, zinc, cadmium, gold and silver are deposited. The problems of obtaining satisfactory electrodeposits are manifold. Deposits of metal are frequently required to possess one or more properties such as brightness, ductility, refined grain, smoothness and attractive color. Moreover, in the plating process, it is desirable to obtain the desired properties over a substantial current density range. Compounds which improve one or more of these properties of the electrodeposited metal or which provide advantages in the plating process are added to the electrolyte solutions either singly or in combination with other additives.

Accordingly, it is the general object of this invention to provide novel cyanide electrolyte plating baths and processes associated therewith capable of enhancing the brightness, color and smoothness of the electrodeposited metal.

A more specific object of this invention is to provide novel cyanide electrolyte plating baths containing soluble salts derived from the reaction of certain substituted and unsubstituted thioltriazines with certain substituted and unsubstituted primary and secondary amines so that the brightness, color and smoothness of the metal is enhanced over a relatively broad range of current densities.

Yet another object of this invention is to provide novel cyanide electrolyte plating baths containing soluble salts derived from the reaction of certain substituted and unsubstituted thioltriazines with certain substituted and unsubstituted primary and secondary amines in combination with certain polymerized alkyl naphthalene sulfonic acids so that the brightness, color and smoothness of the metal is enhanced over a relatively broad range of current densities for prolonged periods of electrolyte use.

Other and further objects of this invention will, in part, be obvious and will, in part, appear hereinafter.

Briefly, this invention comprises the addition of certain compounds to conventional cyanide electrolyte plating baths to promote brighter and smoother deposits of the metal. These addition agents are the soluble salts derived from the reaction of certain substituted and unsubstituted thioltiazines with certain substituted and unsubstituted primary and secondary amines either alone or in combination with certain polymerized alkyl naphthalene sulfonic acids.

In accordance with this invention and in the attainment of the foregoing objects, it has been discovered that the brightness, smoothness, and leveling of metals deposited from cyanide electrolytes is improved by the addition to

2

the electrolyte of water soluble brightener compounds prepared by reacting (A) at least one compound having the formula:



0 wherein  $R_1$  is a radical selected from the group consisting of hydrogen, thiol, amino and hydroxyl radicals with (B) at least one compound having the formula:



wherein R<sub>2</sub> and R<sub>3</sub> are radicals selected from the group consisting of (1) hydrogen, (2) substituted and unsubstituted aliphatic radicals containing not more than four carbon atoms in which the substituents are selected from the group consisting of —NH<sub>2</sub>, —C1, —OH and —SO<sub>3</sub>Na, (3) substituted and unsubstituted alicyclic radicals containing from 4 to 6 carbon atoms in which the substituents are selected from the group consisting of —NH<sub>2</sub>, —C1, —OH and —SO<sub>3</sub>Na and (4) substituted and unsubstituted heterocyclic radicals containing 5 to 6 ring atoms selected from the group consisting of C, S, N and O atoms at least three of which are C atoms and in which the substituents are selected from the group consisting of NH<sub>2</sub>, C1, OH and —SO<sub>3</sub>Na.

Examples of suitable compounds described by the Formula A hereinabove, referred to hereinafter as thiatriazine compounds for convenience, include dithioamamide, dithiocyanuric acid, 2-methyl-s-triazine-4-6-dithiol, 2,4-s-triazinedithiol and trithiocyanuric acid.

Examples of compounds which may be employed in the reaction with the described thio-triazine compounds include methylalamine, 2-chloroethylamine, 1,4-diaminobutane, ethylamine, the sodium salt of 3-amino-n-propylsulfonic acid, methylethylamine, (aminoethyl) ethylamine, diethanolamine, methylhydroxymethylamine, di(chloropropyl) amine, aniline, chloroaniline, p-aminobenzenesulfonate, diphenylamine, 2-hydroxycyclobutetyl phenyl amine, methyl phenyl amine, 3-hydroxyethylaminobenzene sulfonic acid sodium salt, di(p-aminophenyl) amine, chloromethylaniline, diethylenetriamine, 2-aminothiazole, pyridine, pyridine-3-sulfonic acid salt, 2-methylaminopyrrole, 3-aminopyridine, 2,4-dihydroxypyridine, 2-amino-5-chlorofuran, 3,5-dichloropyridine, and guanine. It is apparent that these compounds are described by the Formula B hereinabove. For convenience, these compounds will be referred to hereinafter as the amino compounds.

The described amino compounds are sufficiently strong bases so that they will react with the hydrogen of the thiol radical of the thiol-triazine compound to form a salt therewith. It is apparent that the described thiol-triazine compounds may contain two or three thiol groups. One to three moles of the amino compounds may be employed to react with the thiol groups.

Obviously, in products resulting from the reaction of amines with these thioltriazines all of the thiol groups

are not necessarily reacted. If, for example, only one mole of an amine is reacted with trithiocyanuric acid it is apparent that all of the thiol groups would not be reacted.

It is to be understood that dithioammelide exists as an intramolecular salt. The amine group of the dithioammelide is basic enough to react with a thiol group on another molecule of dithioammelide. The formula outlined hereinabove in the case of dithioammelide then, should be considered to be an empirical formula, the intramolecular salt being a dimer or polymer of this formula. Obviously, in this intramolecular salt, only one thiol group of the dithioammelide is available for further reaction with an amine.

While other reaction mediums for the preparation of the brightener compounds may be employed, either water and/or lower alkyl alcohols having up to 4 carbon atoms are preferred as the solvent or reaction medium. Alkylolamines are the preferred amino compounds because they produce brightener or salt compounds which are among the most soluble.

These water soluble salt compounds, which are employed in this invention as brighteners in metal cyanide electrolytes, and the processes for preparing these salt compounds, are disclosed and claimed in U.S. application Serial No. 260,896 filed February 25, 1963, which is assigned to the assignee of this invention. Reference is made thereto for details and specific examples of the preparation of these compounds. It is to be understood that for convenience, these water soluble salts may be referred to as reaction product additives.

The thioltriazine compounds, described as reactants in detail heretofore, may also be described as thiol substituted heterocyclic ring compounds in which the ring members comprise alternating carbon and nitrogen atoms, in which at least two of the ring carbons carry a thiol substituent. As described hereinabove, the amino compound will, according to this invention, react with at least one of the thiol substituents to produce a salt therewith. Thus, the salt products of this invention may be described as water soluble substituted heterocyclic ring compounds in which the ring members comprise alternating carbon and nitrogen atoms in which at least one ring carbon carries a substituent having the general formula:



wherein R<sub>4</sub> and R<sub>5</sub> are radicals selected from the group consisting of (1) hydrogen, (2) substituted and unsubstituted aliphatic radicals containing not more than four carbon atoms in which the substituents are selected from the group consisting of —NH<sub>2</sub>, —Cl, —OH and —SO<sub>3</sub>Na, (3) substituted and unsubstituted alicyclic radicals containing from 4 to 6 carbon atoms in which the substituents are selected from the group consisting of —NH<sub>2</sub>, —Cl, —OH and —SO<sub>3</sub>Na and (4) substituted and unsubstituted heterocyclic radicals containing 5 to 6 ring atoms selected from the group consisting of C, S, N and O atoms at least three of which are C atoms and in which the substituents are selected from the group consisting of —NH<sub>2</sub>, —Cl, —OH and —SO<sub>3</sub>Na. It is to be understood, of course, that other ring carbon atoms may also be so substituted or they may carry a radical selected from the group consisting of hydrogen, methyl, amino, hydroxyl and thiol radicals. In any event, at least 2 carbon atoms shall be bound to sulfur atoms.

It has also been discovered that the brightness of a metal deposited from the described cyanide electrolyte may be even further enhanced by also adding organic materials such as the sodium and potassium salts of polymerized alkyl naphthalene sulfonic acids. These

auxiliary brighteners may be described as the sodium and potassium salts of compounds having the formula:



wherein R is selected from the group consisting of methyl and ethyl radicals and n is from 1 to about 100. The use of the polymerized alkyl naphthalene sulfonic acids, in conjunction with other compounds, is disclosed, for example, in U.S. Patents 2,701,234, 2,774,728, 2,841,542, 2,861,929 and 2,970,951. In conjunction with the described reaction product brightener compounds, the auxiliary brightener also increases the bright current density range, improves anode corrosion so that less anode polarization occurs and prolongs the active life of the brightener compound. These compounds may be referred to as auxiliary additives, for convenience.

In order to indicate even more fully the advantages and capabilities of the present invention, the following specific examples are set forth to illustrate the utilization of the reaction product additive brightener compounds and auxiliary additive brightener compounds in cyanide metal plating baths.

#### Example I

An aqueous electroplating electrolyte of the following composition was prepared:

|                                                       | Oz./gal. |
|-------------------------------------------------------|----------|
| Copper                                                | 6.0      |
| KOH                                                   | 5.0      |
| Free KCN                                              | 1.2      |
| Reaction product of dithioammelide and 2-aminoethanol | 0.008    |

This bath was operated at a temperature of 165° F. with air agitation. Copper was plated on rectangular steel panels from the bath using a periodic reverse current having a plate time of 5 seconds and a deplating time of 1 second, the reverse current being 100% of the plating current. An excellent smooth and bright copper deposit was obtained over a current density range up to 100 a.s.f. Increasing the amount of the reaction product to 0.02 oz./gal. in the bath resulted in bright deposits over a current density range up to 90 a.s.f. Panels plated from the bath using interrupted direct current and direct current methods showed a bright range up to 50 a.s.f.

#### Example II

An aqueous bath of the following composition was operated at 165° F. with air agitation to plate steel panels.

|                                                          | Oz./gal. |
|----------------------------------------------------------|----------|
| Copper                                                   | 6.0      |
| KOH                                                      | 5.0      |
| Free KCN                                                 | 1.2      |
| Reaction product of dithioammelide and 2-aminoethanol    | 0.01     |
| Sodium salt of polymerized naphthalene bis-sulfonic acid | 0.006    |

Using the periodic reverse current cycle described in Example I produced copper deposits with an enhanced brightness over a current density range up to 90 a.s.f. With direct current methods, the enhanced brightness range extended up to 60 a.s.f.

#### Example III

An aqueous bath of the following composition was operated at 180° C. to plate steel panels using a periodic reverse current process having a plating time of 60 seconds and a deplating time of 40 seconds, the reverse current being 50% of the plating current.

|                                                          | Oz./gal. |
|----------------------------------------------------------|----------|
| KOH                                                      | 5.0      |
| Free KCN                                                 | 1.2      |
| NaCNS                                                    | 0.3      |
| ZnO                                                      | 0.06     |
| Reaction product of dithioammelide and 2-aminoethanol    | 0.03     |
| Sodium salt of polymerized naphthalene bis-sulfonic acid | 0.006    |

This bath produced excellent bright leveled copper deposits. The same bath without the reaction product and the sodium salt produced a hazy bright deposit.

#### Example IV

Aqueous baths of the following compositions were employed in a series of tests in a Hull Cell with additives known in the art and an additive of this invention at various concentrations of each. All of the baths were operated at 180° F. with air agitation.

|                                                           | Oz./gal. |
|-----------------------------------------------------------|----------|
| Basic bath:                                               |          |
| Copper                                                    | 6.0      |
| Free KCN                                                  | 1.2      |
| KOH                                                       | 5.0      |
| Additives to basic bath:                                  |          |
| 1A. Diethioammelide                                       | 0.005    |
| 1B. Dithioammelide                                        | 0.005    |
| 2-aminoethanol                                            | 0.002    |
| 1C. Reaction product of dithioammelide and 2-aminoethanol | 0.005    |
| 2A. Dithioammelide                                        | 0.05     |
| 2B. Dithioammelide                                        | 0.05     |
| 2-aminoethanol                                            | 0.04     |
| 2C. Reaction product of dithioammelide and 2-aminoethanol | 0.05     |
| 3A. Dithioammelide                                        | 0.10     |
| 3B. Dithioammelide                                        | 0.10     |
| 2-aminoethanol                                            | 0.04     |
| 3C. Reaction product of dithioammelide and 2-aminoethanol | 0.10     |

A total of 18 test panels were prepared in order to compare the effect of the three additive systems at various concentrations. Nine panels were prepared using a periodic reverse current process having a plating time of 5 seconds and a deplating time of 1 second, the reverse current being equal to the plating current. Nine panels were prepared using a direct current. The Hull Cell panels were examined and the bright current density ranges are reported in Table I.

TABLE I.—BRIGHT CURRENT DENSITY RANGES ON HULL CELL PANELS IN A.S.F.

| Additive System | PR Panels    | DC Panels    |
|-----------------|--------------|--------------|
| 1A              | 35-120       | 0-35         |
| 1B              | 0-70         | 0-20, 70-140 |
| 1C              | 0-120        | 38-80        |
| 2A              | 0-20, 55-130 | 0-10, 30-110 |
| 2B              | 0-40         | 0-20, 40-80  |
| 2C              | 0-130 a.s.f. | 0-18, 36-110 |
| 3A              | 0-15, 55-140 | 0-18, 60-130 |
| 3B              | 0-15, 55-140 | 0-18, 60-130 |
| 3C              | 0-140        | 0-30, 50-130 |

It is apparent from the data presented in Table I that the brightness and current density ranges from the baths containing the reaction product additive are superior to the baths containing dithioammelide alone or the unreacted dithioammelide in combination with 2-aminoethanol.

#### Example V

An aqueous bath of the following composition was operated at 165° F. with air agitation to plate Hull Cell panels at 3 amperes using the periodic reverse current cycle described in Example IV.

|                                                                 | Oz./gal. |
|-----------------------------------------------------------------|----------|
| Copper                                                          | 6.0      |
| Free KCN                                                        | 1.2      |
| KOH                                                             | 5.0      |
| 5 NaCNS                                                         | 0.4      |
| ZnO                                                             | 0.06     |
| Reaction product of dithiocyanuric acid and methylchloroaniline | 0.01     |

10 A bright copper deposit was obtained in a current density range of 0-130 a.s.f. Increasing the reaction product concentration to 0.2 oz./gal. shortened the bright current density range to 0-100 a.s.f.

#### Example VI

15 An aqueous bath of the following composition was operated at 180° F. to plate Hull Cell panels using the periodic reverse current cycle described in Example IV.

|                                                             | Oz./gal. |
|-------------------------------------------------------------|----------|
| 20 Copper                                                   | 6.0      |
| Free KCN                                                    | 1.2      |
| KOH                                                         | 5.0      |
| Reaction product of trithiocyanuric acid and di-methylamine | 0.015    |

25 A bright copper deposit was obtained in a current density range of 0-50 a.s.f. Adding 0.06 oz./gal. of ZnO and 0.01 oz./gal. of the potassium salt of polymerized naphthalene bi-sulfonic acid enhanced the brightness and increased the range to 0-110 a.s.f. No appreciable benefit was noted from further additions of the reaction product.

#### Example VII

30 35 An aqueous bath of the following composition was operated at 165° F. with air agitation of plate Hull Cell panels employing an interrupted direct current.

|                                                                                               | Oz./gal. |
|-----------------------------------------------------------------------------------------------|----------|
| 40 Copper                                                                                     | 6.0      |
| Free KCN                                                                                      | 1.2      |
| KOH                                                                                           | 5.0      |
| ZnO                                                                                           | 0.06     |
| NaCNS                                                                                         | 0.4      |
| 45 Reaction product of 2-methyl-s-triazine-4,6-thiol with 2-aminothiazole and 3-aminopyridine | 0.010    |

50 A bright range of 0-85 a.s.f. was observed on the panel. Adding 0.002 oz./gal. of the sodium salt of polymerized naphthalene bis-sulfonic acid enhanced the brightness but the bright current density range was reduced to 0-75 a.s.f.

#### Example VIII

55 An aqueous bath of the following composition was operated at 175° F. with air agitation to plate Hull Cell panels employing the period reverse cycle of Example IV.

|                                                                 | Oz./gal. |
|-----------------------------------------------------------------|----------|
| Copper                                                          | 8.3      |
| Free NaCN                                                       | 2.0      |
| 60 NaOH                                                         | 4.0      |
| Na <sub>2</sub> CO <sub>3</sub>                                 | 10.1     |
| Reaction product of trithiocyanuric acid and methylethanolamine | 0.008    |

65 A bright range of about 0-100 a.s.f. was observed on the panel. The addition of the sodium salt of polymerized naphthalene bis-sulfonic acid produced a sample with more depth of color in the bright range.

#### Example IX

70 75 This example was identical to Example VIII, except that 0.015 oz./gal. of the reaction product of s-triazine-2,4-dithiol and n-butylamine was employed as the brightener. Results substantially identical to that of Example VIII were observed.

## Example X

An aqueous bath of the following composition was operated at 100° F. at room temperature to plate Hull Cell panels employing a periodic reverse current having a plating time of 20 seconds and a deplating time of 2 seconds, the reverse current being 100% of the plating current.

|                                                                           | Oz./gal. |
|---------------------------------------------------------------------------|----------|
| Free NaCN                                                                 | 7.0      |
| CuCN                                                                      | 2.4      |
| ZnCN                                                                      | 5.1      |
| KOH                                                                       | 6.9      |
| Cu/Zn Ratio: 0.6 (reaction product of dithioam-melide and 2-aminoethanol) | 0.10     |

A bright range from 0 to 100 a.s.f. was observed on the panel of deposited white brass. It was also observed that the white brass anodes were brightened, resulting in better anode corrosion. Addition of 0.003 oz./gal. of the sodium salt of polymerized naphthalene bis-sulfonic acid produced brighter deposits from 0-120 a.s.f.

In aqueous baths and processes identical to that described in Example IX except that another reaction product was employed, substantially equivalent results were obtained with the reaction product of dithiocyanuric acid and sodium aminobenzene-sulfonate.

At least 0.005 ounce of the reaction product additive compound should be added for each gallon of the aqueous metal cyanide bath, preferably from 0.008 to 0.2 ounce per gallon of bath. At least 0.001 ounce of the auxiliary brightener should be added for each gallon of the bath when the combined reaction product and auxiliary brightener system is to be employed. The maximum concentration of either the reaction product additive or the auxiliary additive is limited only by the solubility of the particular compound in the bath. With high concentration of the auxiliary additive, a striated deposit of metal may be produced. These striations can be eliminated by increasing the free cyanide content of the bath.

The described reaction product additives and the described auxiliary additives may be used in further combination with other known additives for cyanide electroplating baths, as for example together with zinc oxide and sodium thiocyanate. This particular combination provides a particularly prolonged active life for the brightener compounds.

Aqueous alkaline metal cyanide electroplating baths are well-known in the art. Metals which fall within the scope of this invention include, for example, copper, brass and zinc. The aqueous cyanide plating baths will contain soluble compounds of at least one of the metals selected from the group consisting of copper and zinc. The make-up of these baths is disclosed in the patent literature and also in standard texts or handbooks, as for example the Metal Finishing Guidebook Directory, 30th Ed., 1962, published by Metals and Plastics Publications, Inc., Westwood, New Jersey.

While the present invention has been described with particular reference to preferred embodiments thereof, it will be understood, of course, that certain changes, substitutions, modifications and the like may be made therein without departing from its true scope.

I claim as my invention:

1. An aqueous alkaline cyanide metal plating solution containing a metal cyanide from the group consisting of copper cyanide and mixtures of copper cyanide and zinc cyanide, an alkali cyanide and an effective amount sufficient to impart brightness of water soluble salt formed from (A) at least one compound having the formula



wherein  $\text{R}_1$  is a radical selected from the group consisting of hydrogen, thiol, amino and hydroxyl radicals and (B) at least one compound having the formula



wherein  $\text{R}_2$  and  $\text{R}_3$  are radicals selected from the group consisting of (1) hydrogen, (2) substituted and unsubstituted aliphatic radicals containing not more than four carbon atoms in which the substituents are selected from the radicals consisting of  $-\text{NH}_2$ ,  $-\text{Cl}$ ,  $-\text{OH}$  and  $-\text{SO}_3\text{Na}$ , (3) substituted and unsubstituted carbocyclic radicals containing from 4 to 6 ring carbon atoms in which the substituents are selected from the radicals consisting of  $-\text{NH}_2$ ,  $-\text{Cl}$ ,  $-\text{OH}$  and  $-\text{SO}_3\text{Na}$  and (4) substituted and unsubstituted heterocyclic radicals containing 5 to 6 ring atoms selected from the group consisting of C, S, N and O atoms at least three of which are C atoms and in which the substituents are selected from the group consisting of  $-\text{NH}_2$ ,  $-\text{Cl}$ ,  $-\text{OH}$  and  $-\text{SO}_3\text{Na}$ .

2. An aqueous alkaline cyanide metal plating solution containing a metal cyanide from the group consisting of copper cyanide and mixtures of copper cyanide and zinc cyanide, an alkali cyanide and an effective amount sufficient to impart brightness of water soluble salt formed from (A) at least one compound selected from the group consisting of dithiocyanuric acid, dithioam-melide, 2-methyl-s-triazine-4,6-dithiol, 2,4-s-triazinedithiol and trithiocyanuric acid and (B) at least one compound selected from the group consisting of methylolamine, 2-aminoethanol, 2-chloroethylamine, 1,4-diaminobutane, ethylamine, the sodium salt of 3-amino-n-propylsulfonic acid, methylethylamine, (aminoethyl) ethylamine, diethylolamine, methylhydroxymethylamine, di(chloropropyl)amine, aniline, chloroaniline, p-aminoaniline, 3-hydroxycyclopentylamine, 3-aminobenzenesodiumsulfonate, diphenylamine, 2-hydroxycyclobutetyl phenyl amine, methyl phenyl amine, 3-hydroxyethylaminobenzene sulfonic acid sodium salt, di(p-aminophenyl)amine, chloromethyl aniline, diethylenetriamine, 2-aminothiazole, pyridine, pyridine-3-sulfonic acid salt, 2-methylaminopyrrole, 3-aminopyridine, 2,4-dihydroxypyridine, 2-amino-5-chlorofuran, 3,5-dichloropyridine, and guanidine.

3. In the process of plating copper or both copper and zinc on a metal base member from an aqueous alkaline metal cyanide bath containing a metal cyanide from the group consisting of copper cyanide and both copper cyanide and zinc cyanide, the improvement which comprises electrodepositing said metal from said bath to which has been added an effective amount sufficient to impart brightness of a water soluble salt formed from (A) at least one compound having the formula



wherein  $\text{R}_1$  is a radical selected from the group consisting of hydrogen, thiol, amino and hydroxyl radicals and (B) at least one compound having the formula



75 wherein  $\text{R}_2$  and  $\text{R}_3$  are radicals selected from the group

consisting of (1) hydrogen, (2) substituted and unsubstituted aliphatic radicals containing not more than four carbon atoms in which the substituents are selected from the radicals consisting of  $-\text{NH}_2$ ,  $-\text{Cl}$ ,  $-\text{OH}$  and  $-\text{SO}_3\text{Na}$ , (3) substituted and unsubstituted carbocyclic radicals containing from 4 to 6 ring carbon atoms in which the substituents are selected from the radicals consisting of  $-\text{NH}_2$ ,  $-\text{Cl}$ ,  $-\text{OH}$  and  $-\text{SO}_3\text{Na}$  and (4) substituted and unsubstituted heterocyclic radicals containing 5 to 6 ring atoms selected from the group consisting of C, S, N and O atoms at least three of which are C atoms and in which the substituents are selected from the group consisting of  $-\text{NH}_2$ ,  $-\text{Cl}$ ,  $-\text{OH}$  and  $-\text{SO}_3\text{Na}$ .

4. The aqueous alkaline cyanide metal plating solution of claim 1, in which at least 0.005 ounce of the added compound is dissolved per gallon of solution.

5. The aqueous alkaline cyanide metal plating solution of claim 1, in which from 0.008 to 0.2 ounce of the added compound is dissolved per gallon of solution.

6. The aqueous alkaline cyanide metal plating solution of claim 1, also containing an auxiliary brightener selected from the group of sodium and potassium salts of compounds having the formula:



wherein R is selected from the group consisting of methyl and ethyl radicals and n is from 1 to about 100.

7. The aqueous alkaline cyanide metal plating solution of claim 6, containing at least 0.001 ounce of the auxiliary brightener per gallon of solution.

8. The aqueous alkaline cyanide metal plating bath of claim 1 in which the metal of the metal cyanide is copper.

9. The aqueous alkaline cyanide metal plating bath of claim 1 in which a mixture of copper and zinc cyanides is used.

10. The aqueous alkaline cyanide metal plating solution of claim 2, in which at least 0.005 ounce of the added compound is dissolved per gallon of solution.

11. The aqueous alkaline cyanide metal plating solution of claim 2, also containing an auxiliary brightener added compound is dissolved per gallon of solution.

12. The aqueous alkaline cyanide metal plating solution of claim 2, also containing an auxiliary brightener

selected from the group of sodium and potassium salts of compounds having the formula:



wherein R is selected from the group consisting of methyl and ethyl radicals and n is from 1 to about 100.

13. The aqueous alkaline cyanide metal plating solution of claim 12, containing at least 0.001 ounce of the auxiliary brightener per gallon of solution.

14. The aqueous alkaline cyanide metal plating bath of claim 2 in which the metal of the metal cyanide is copper.

15. The aqueous alkaline cyanide metal plating bath of claim 2 in which a mixture of copper and zinc cyanides is used.

16. The aqueous alkaline cyanide metal plating bath of claim 2 in which the water soluble compound is the product of the reaction of dithioammelide and 2-aminoethanol.

17. The aqueous alkaline cyanide metal plating bath of claim 2 in which the water soluble compound is the product of the reaction of trithiocyanuric acid and methylethanolamine.

18. The aqueous alkaline cyanide metal plating bath of claim 2 in which the water soluble compound is the product of the reaction of dithiocyanuric acid and methylchloroaniline.

19. The aqueous alkaline cyanide metal plating solution of claim 12 also containing zinc oxide and sodium thiocyanate.

**References Cited by the Examiner**  
**UNITED STATES PATENTS**

|           |         |                   |       |        |
|-----------|---------|-------------------|-------|--------|
| 2,609,339 | 9/1952  | Passal            | ----- | 204-52 |
| 2,774,728 | 12/1956 | Wernlund          | ----- | 204-52 |
| 2,841,542 | 7/1958  | Manquen           | ----- | 204-52 |
| 2,849,352 | 8/1958  | Kirstahler et al. | ----- | 204-44 |
| 2,862,861 | 12/1958 | Moy               | ----- | 204-52 |
| 2,970,951 | 2/1961  | Manquen et al.    | ----- | 204-52 |
| 3,018,232 | 1/1962  | Bishoff et al.    | ----- | 204-44 |

JOHN H. MACK, Primary Examiner.

G. KAPLAN, Assistant Examiner.

UNITED STATES PATENT OFFICE  
CERTIFICATE OF CORRECTION

Patent No. 3,296,101

January 3, 1967

James R. Crain

It is hereby certified that error appears in the above numbered patent requiring correction and that the said Letters Patent should read as corrected below.

Column 5, before line 2, insert the following ingredient:

Copper ----- 8.0

same column 5, line 27, for "Diethiomelide" read --  
Dithioammelide --; column 6, line 28, for "bi-sulfonic"  
read -- bis-sulfonic --; line 36, for "of" read -- to --.

Signed and sealed this 3rd day of October 1967.

(SEAL)

Attest:

ERNEST W. SWIDER  
Attesting Officer

EDWARD J. BRENNER  
Commissioner of Patents